

# UNITED STATES PATENT OFFICE.

GEORG EGLY, OF TREPTOW, GERMANY, ASSIGNOR TO GEBRUEDER SIEMENS & CO., OF BERLIN, GERMANY, A CORPORATION OF GERMANY.

## ELECTRIC HEATER.

1,103,353.

Specification of Letters Patent.

Patented July 14, 1914.

No Drawing.

Application filed April 8, 1913. Serial No. 759,803.

*To all whom it may concern:*

Be it known that I, GEORG EGLY, a citizen of the German Empire, and residing at Treptow, near Berlin, Germany, have invented certain new and useful Improvements in Electric Heaters, of which the following is a specification.

My invention relates to electric heaters composed of non-metallic resistance materials. Heaters consisting of non-metallic resistance materials, *e. g.* silit, are preferably made more conductive at the places to which the current is supplied, and at the places adjacent thereto, by means of a metallic coating or by impregnation with metals. Coatings of silver are principally employed for the purpose. The heaters are usually porous and the metal penetrates more or less deeply into them. The coatings not only cause better contact but, owing to their greater conductivity, lessen the glow in the vicinity of the contact-pieces and protect the latter from being burnt. It has however been found that such metallic coatings melt when the temperature is high, and that they gradually recede toward the contact-pieces, toward which the glow therefore continually advances.

A primary object of my invention is to obviate this defect. To this end, I coat that part of the heater which is coated or impregnated with a metal with a glaze such as boracic acid, borates or the like. The effect of this glaze is surprising; the metal entirely ceases to recede, the glow no longer advances along the heater, and the heater remains practically unchanged although its temperature may be considerably above that of the melting point of the metallic coating. It is difficult to assign a reason for the action of the glaze. It is possible

that changes in the conduction and radiation of the heat play some part. Perhaps the glaze in some way directly either prevents the molten metal from shrinking together, or prevents it from exuding from the pores of the heater. The heaters are as a rule porous, and when treated with the metal, the latter penetrates more or less deeply into the interior of the same. When the glaze is lacking, the metal seems to exude from the pores of the heater and to collect in small lumps which gradually recede before the glow. Under the protection of the glaze the metal no longer exudes or forms small globules.

In order to obtain a satisfactory result, it is preferable to melt the glaze slowly on the part containing the metal, so that it can penetrate well into the pores of the heating element.

I claim:

1. An electric heater composed of a non-metallic, highly refractory resistance material provided in the vicinity of the places at which current is supplied with a metallic coating and with a glaze on the metallic coating, for the purpose specified.

2. An electric heater composed of a non-metallic, highly refractory resistance material provided in the vicinity of the places at which current is supplied with a metallic coating glazed with a compound of boron, for the purpose specified.

In testimony whereof, I have signed my name to this specification in the presence of two witnesses.

GEORG EGLY.

Witnesses:

HENRY HASPER,  
WOLDEMAR HAUPT.